

Nov. 13, 1928.

1,691,725

J. W. LEIGHTON

METHOD OF PRODUCING METAL TUBES

Filed Sept. 30, 1926



*Inventor.*

John Wycliffe Leighton.

by  
*H. S. Denison*  
atty.

Patented Nov. 13, 1928.

1,691,725

# UNITED STATES PATENT OFFICE.

JOHN WYCLIFFE LEIGHTON, OF PORT HURON, MICHIGAN.

## METHOD OF PRODUCING METAL TUBES.

Application filed September 30, 1926. Serial No. 138,675.

The principal objects of the invention are, to enable the production of metal tubes by extrusion in large quantities and at low cost, and to devise a simple and effective means 5 for extruding metal billets.

The principal feature of the invention consists in the novel method of partly extruding the metal of the billet from a die and completing the operation by the progressive 10 extrusion of a portion of the succeeding billet.

In the drawings, Figure 1 is an elevational part sectional view of a set of dies showing a partly extruded billet and a heating torch arranged to apply heat to the partly 15 extruded billet.

Figure 2 is an elevational part sectional view of a set of dies showing a succeeding billet placed therein upon a partly extruded billet.

Figure 3 is an elevational part sectional view of the dies showing the succeeding billet partly extruded and completing the extrusion of the preceding billet.

In the manufacture of short length tubing from prepared billets by extrusion methods, numerous forms have been devised but difficulties have been encountered in the maintenance of the tools and in proper clearing of the dies after each operation. The 30 present method overcomes the objections that have been met with.

In the method of extruding billets to form tubes it has been found necessary to form the die with a bevelled bottom wall so that the metal may flow smoothly into the smaller 35 diameter orifice. It is impossible to construct a punch which will successfully perform the operation of extruding the material of the billet through the finishing orifice.

According to the present method the die 1 is formed with a recess 2 of a diameter slightly greater than the billets that are used.

The bottom wall 3 of this die converges to the diameter of the orifice 4 which is the full diameter of the finished tube.

The billets 5 used are of cylindrical form and they have a central orifice therethrough 50 which is substantially the same size as the inner diameter of the finished tube.

The punch 7 is of the same diameter as the recess 2 and is adapted to fit snugly thereinto and centrally arranged in the punch 7 and extending from the lower end thereof

is a pilot 8 which is the same diameter as the inner diameter of the finished tube and is adapted to extend axially through the orifice 4 to form a throat through which the metal of the billet is forced.

In the forming of a length of tube in this die a heated billet is placed in the die and the punch is moved downwardly until the pilot extends through the central orifice thereof and the end of the punch closes the die recess, the pilot extending into the orifice 4.

A continued movement of the punch causes the metal of the billet to flow around the pilot and inwardly in the convergent die 70 recess to the throat surrounding the pilot.

The method thus forms a tube of the desired diameter and thickness.

The punch which is shown square across the bottom end in order to obtain the proper 75 result in the flowing of the metal of the billet, cannot follow the metal past the upper shoulder of the tapered end of the recess, consequently the metal is not completely extruded.

An annular recess 9 is formed in the side wall of the die recess which retains a narrow rib of the upper edge of the metal of the partly extruded tube and this rib of metal forms a positive lock to hold the partly 80 finished tube in the die allowing the withdrawal of the punch and its pilot clear therefrom.

After the punch has been withdrawn a suitable torch 10 swings over the die recess 90 and a flame is directed downwardly against the upper end of the partly extruded tube. This flame which may be very hot is continued for a sufficient length of time to maintain the desired temperature of the upper 95 part of the metal and the torch is then withdrawn and another heated billet is dropped into the die. The punch then descends into the die and the force exerted against the billet first causes the metal of the former billet 100 to flow until the tube is completely extruded. The punch continuing further to descend causes the next billet to be extruded in a similar manner to the foregoing one.

The process thus described is continued indefinitely, each billet being reheated in the die following the initial extrusion of the major portion thereof.

This method of manufacturing short length tubes has proven to be very successful 110

and the cost of manufacture is reduced to the minimum.

What I claim as my invention is:—

1. A method of extruding metal tubes,
- 5 consisting in placing a heated billet in a die, then partly extruding the same from the die, by means of a punch, then withdrawing the punch, leaving the partly extruded billet in place, then reheating the unextruded portion  
10 of the metal, then placing a heated billet in the die above said reheated unextruded portion and returning the punch into the die against said heated billet to complete the extrusion of the preceding tube and effect the  
15 partial extrusion of said heated billet.

2. A method of extruding metal tubes,

consisting in placing a heated billet within a die having a tapering throat, then applying pressure to force the metal of the billet through the throat, then directing a flame into the die to impinge against the unextruded end of the billet, then inserting another heated billet on the top of the unextruded portion of the former billet, then applying pressure to the latter billet to force the heated extruded metal of the preceding billet through the throat of the die to complete the extrusion of the first mentioned billet and effect a partial extrusion of the following billet.

JOHN WYCLIFFE LEIGHTON.